

Dec. 8, 1931.

F. D. LEWIS  
MANUFACTURE AND PRODUCTION OF ARTIFICIAL  
THREADS, FILAMENTS, AND THE LIKE  
Filed May 26, 1927

1,835,956



FREDERICK DONALD LEWIS

by his attorneys

Howson and Howson

## UNITED STATES PATENT OFFICE

FREDERICK DONALD LEWIS, OF LITTLEBOROUGH, MANCHESTER, ENGLAND, ASSIGNOR  
TO COURTAULDS LIMITED, OF LONDON, ENGLAND

MANUFACTURE AND PRODUCTION OF ARTIFICIAL THREADS, FILAMENTS AND  
THE LIKE

Application filed May 26, 1927, Serial No. 194,527, and in Great Britain July 19, 1926.

This invention relates to the production of artificial threads, filaments or the like by a dry spinning process in which a solution of a cellulose ester or cellulose ether in a volatile solvent is projected through minute orifices into a warm atmosphere, in such manner that the volatile solvent is evaporated, leaving the cellulose derivative in the form of filaments or threads.

10 When the nozzle, through which the spinning solution is projected, is situated inside the chamber or cell through which a current of hot air is passing, a certain amount of heating of the spinning solution takes place before it passes through the nozzle. Further, it has been proposed to heat the spinning solution before the extrusion in order to reduce the viscosity of the said solution and also to enable the evaporation of the solvent to take place more quickly. It has also been proposed to regulate the temperature in the neighbourhood of the spinning nozzle in a manner independent of the temperature of the remainder of the chamber or cell, and in this connection it has been proposed, on the one hand to maintain the nozzles at a low temperature, and on the other hand to effect a definite input of heat in the region of the spinning nozzles, for instance, by preheating the spinning solution on its way to the nozzle. In either of these latter cases, however, the temperature maintained at the spinning nozzles, and in the zone immediately in their neighbourhood, is adjustable and variable, and is independent of the temperature of the remainder of the cell.

20 I have now found that considerable advantages are obtained in the process of dry spinning of solutions of cellulose esters or cellulose ethers if the solution at the spinning nozzle and the air in that part of the spinning chamber which is in the neighbourhood of the nozzle be maintained at practically the same temperature by subjecting both the said solution and the whole of the air in the spinning chamber to the action of the same supply of heat, so that the temperature at the spinning nozzle and in the zone immediately in its neighbourhood is dependent on the temperature of the remainder of

the cell. The two temperatures, that is to say, of the solution at the spinning nozzle and of the air in the chamber, are thus dependent one upon the other. It is very important that the conditions obtaining during 55 the production of artificial filaments by the dry spinning process should be strictly under control, and the fact that, according to the present invention, two of the essential temperatures can be made to depend one upon 60 the other in this manner constitutes an important advantage of the process according to the present invention.

25 The heating of the spinning solution to the same temperature as that of the air in 65 the spinning chamber according to this invention can be effected according to various methods. For example, the spinning solution may pass through a pipe which traverses practically the whole length of the 70 spinning chamber before it reaches the nozzle so that as the spinning solution passes through this pipe, it gradually attains the same temperature as that of the air in the adjacent to the nozzle; or the pipe through 75 which the spinning solution passes may take the form of a coiled pipe or a spiral situated at the upper end of the spinning chamber adjacent to the nozzle; or the pipe through 80 which the spinning solution passes may be led through the hot water jacket surrounding the spinning chamber and thence pass to the spinning nozzle. It is, however, essential that the length of the said pipe situated in the spinning chamber or in the water jacket 85 thereof, be sufficiently great to ensure that the spinning solution, when it reaches the spinning nozzle, shall have attained a temperature equal to that of the air in the spinning chamber. Another method consists in 90 passing the solution through a suitable pipe situated in a vessel through which passes the whole of the hot water leaving the hot water jacket of the spinning chamber. If in any of the foregoing arrangements the supply of 95 hot water to the jacket of the spinning chamber be varied in order to vary the temperature of the air in the spinning chamber, a corresponding variation in the temperature 100 of the spinning solution will be effected.

The accompanying drawings illustrate diagrammatically in vertical cross-section, examples of apparatus suitable for use in the manufacture and production of artificial threads, filaments, and the like, in accordance with this invention, but it is to be understood that the said invention is not restricted to the examples of apparatus shown. In each of the said examples A is the spinning nozzle situated inside a spinning chamber B, the said spinning chamber being surrounded by a jacket C and so arranged that hot water can be circulated in the space between B and C, entering by the pipe D and leaving by the pipe E. In Figure 1, the top part of the spinning chamber is shown as a hollow space, through which the hot water circulates, while in Figures 2, 3 and 4 the spinning chamber is closed at the top by a plate F. The air enters each spinning chamber through an opening G at the lower end, and leaves through a pipe H at the top. In Figure 1 the spinning solution is led through a long pipe K, which traverses practically the whole length of the spinning chamber before it reaches the spinning nozzle A.

In the modification shown in Figure 2, the spinning solution passes through a coiled or spiral pipe L situated in the upper part of the spinning chamber adjacent to the spinning nozzle A.

In the modification shown in Figure 3 the spinning solution passes through a pipe M which is situated in the hot water in the space between the chamber B and the jacket C, and thence to the spinning nozzle A.

In the modification shown in Figure 4, the spinning solution on its way to the nozzle A, is heated by being passed through a coil N, which is situated in a vessel O through which passes the whole of the water leaving the hot water jacket of the spinning chamber.

I have also found that the process of employing a common temperature of the spinning solution and of the air in the spinning chamber according to the present invention possesses a further advantage in that it affords an accurate control of the variation of the lustre of the filaments produced, so that the said lustre can be augmented or diminished at will.

Generally speaking, for any concentration of cellulose acetate, in a solvent, if other conditions of spinning be kept constant, there will be a maximum common temperature at which it is possible to obtain continuous filaments; above this maximum temperature either for the reason that the evaporation of the solvent takes place too rapidly or for some other reason, the spinning of a continuous filament is not possible. I have further found that threads of greater lustre and freedom from glitter can be obtained by employing a common temperature at or approaching the said maximum temperature. For exam-

ple, when spinning a 20 per cent solution of cellulose acetate in acetone and controlling the air current through the chamber so that the concentration of the acetone in the vicinity of the nozzle is about 1.5 per cent by volume, filaments of roundish cross-section and great lustre will be obtained by employing a common temperature of 67° centigrade for the spinning solution and the evaporating atmosphere. Maintaining other factors affecting evaporation constant, and lowering the common temperature to 65° centigrade less lustrous threads of roundish cross-section are obtained, and by lowering the temperature still further to 62° centigrade the threads formed are still less lustrous. If the common temperature be reduced to 55° centigrade the cross-section of the filaments obtained will show more or less parallel but curved sides, whereas with a still lower temperature of 35° centigrade the cross-section of the filaments will be flat and straight.

When employing more concentrated solutions of cellulose acetate, for instance 23 per cent or 25 per cent of cellulose acetate in acetone, the maximum common temperature employable for obtaining continuous filaments will be lower than that which can be used with a 20 per cent solution of cellulose acetate. On the other hand, if the current of air through the spinning chamber be controlled so that the percentage of solvent in the neighbourhood of the nozzle is increased, it will generally be necessary to use a higher common temperature in order to obtain the greatest lustre.

As a general rule, if a solvent of lower boiling point be employed for preparing the solution of cellulose acetate, it will be necessary to employ for the purpose of spinning, a lower common temperature of the spinning solution and the spinning chamber. For instance, when spinning a 21 per cent solution of cellulose acetate in a mixed solvent containing 75 per cent acetone and 25 per cent ethyl chloride, the concentration of solvent in the evaporating atmosphere in the vicinity of the nozzle being about 1.5 per cent by volume, threads of roundish cross-section of greater lustre are obtained by spinning at or near the maximum common temperature of about 45° centigrade. Less lustrous threads of roundish cross-section are produced by lowering the common temperature to 40° centigrade if other conditions effecting the evaporation of the solvent are maintained constant.

What I claim is:—

1. In the manufacture and production of artificial threads, filaments and the like from cellulose esters or cellulose ethers by a dry spinning process, the step which consists in subjecting both the said solution for a distance on its way to the spinning nozzle and the whole of the air in the spinning chamber

to the action of the same supply of heat, whereby the temperature of the solution as it leaves the spinning nozzle is practically the same as the temperature of the atmosphere about the nozzle.

5. 2. Apparatus for the spinning of artificial threads, filaments and the like by a dry spinning process, comprising a spinning chamber provided with a heating jacket in combination with a spinning nozzle having a supply pipe which is heated from said heating jacket for a considerable distance leading up to the nozzle sufficient to cause the temperature of the solution as it leaves the spinning nozzle to be practically the same as the temperature of the atmosphere surrounding the nozzle.
10. 3. Apparatus for the spinning of artificial threads, filaments and the like by a dry spinning process, comprising a spinning chamber provided with a heating jacket in combination with a spinning nozzle having a supply pipe traversing practically the whole length of the spinning chamber on its way to the spinning nozzle.
15. 4. Apparatus for the spinning of artificial threads, filaments and the like by a dry spinning process, comprising a spinning chamber provided with a heating jacket in combination with a spinning nozzle having a supply pipe coiled within the heated spinning chamber.

20. 5. Apparatus for the spinning of artificial threads, filaments and the like by a dry spinning process, comprising a spinning chamber provided with a heating jacket in combination with a spinning nozzle having a supply pipe passing through the said jacket on its way to the nozzle within the chamber.

25. In testimony whereof I have signed my name to this specification.

40. **FREDERICK DONALD LEWIS.**

45

50

55

60

65

**CERTIFICATE OF CORRECTION.**

**Patent No. 1,835,956.**

**Granted December 8, 1931, to**

**FREDERICK DONALD LEWIS.**

**It is hereby certified that error appears in the printed specification of the above numbered patent requiring correction as follows: Page 1, line 75, strike out the words "adjacent to the nozzle" and insert instead spinning chamber; and that the said Letters Patent should be read with this correction therein that the same may conform to the record of the case in the Patent Office.**

**Signed and sealed this 9th day of February, A. D. 1932.**

**(Seal)**

**M. J. Moore,  
Acting Commissioner of Patents.**